

## UNITED STATES PATENT OFFICE

2,353,058

## METALLIC PASTE PIGMENT

Leo J. Mitchell, Clayton, Mo.

No Drawing. Application September 18, 1940;  
Serial No. 357,285

12 Claims. (Cl. 260—31)

The so-called bronze powders are familiar commercial products that consist mainly of fine particles of metallic aluminum, copper, zinc or alloy thereof with or without pigments. As a result of the process of grinding or stamping by which they are produced, the particles are in the form of thin flat flakes with one dimension considerably smaller than the others, and these particles bear a minute film of grease, such as stearic acid or palmitic acid, that was mixed with the material as a polishing agent during the process of grinding. So long as the powders thus produced remain in the condition in which they leave the grinder of a stamp mill, they are known as "straight run" bronze powders.

In all, possibly a dozen basic colors are available in these straight-run powders. The range of colors can be greatly enhanced by heat-treating or oxidizing the powders, i. e., either the true bronze powders or the copper powders. The powders progressively become darker as they are exposed to higher temperatures, or to a specific temperature for a longer period of time, or to a combination of both conditions. A few additional shades can be made by treating certain powders with acetic acid.

The effect of heating "straight run" powders is to cause the thin flat flakes thereof to curl and to some extent to adhere or agglomerate together. So long as the flakes are thin and flat, they are well suited for use in varnish and lacquer to produce a smooth coat with a large covering capacity; but when the flakes are curled, they tend to form an uneven coat of greatly reduced covering capacity.

Accordingly, it is the object of the present invention to devise a bronze powder paste which will answer all the requirements which formerly could only be satisfied by the use of a straight run bronze powder in conjunction with a pigmented lacquer and can be made available in many shades which formerly could be obtained only with coarse oxidized bronzes, or by the use of aniline dyed powders. Due to rigid laboratory control in its manufacture the color which my bronze paste yields is always consistent and is not subject to variations such as are likely when other methods are used to arrive at a given color.

The following formula is typical of a dark bronze powder in current use:

|                                              |       |
|----------------------------------------------|-------|
| Graphite                                     | 5.00  |
| Patent red lining (aniline dyed gold powder) | 10.00 |

|                                              |       |
|----------------------------------------------|-------|
| Antique statuary (oxidized rich gold powder) | 20.00 |
| Copper stripping new (straight run copper)   | 15.00 |
| Nigger bronze (oxidized pale gold powder)    | 50.00 |

It is noted that the foregoing bronze powder contains 5 per cent graphite. The presence of this material necessitates extreme care in application as there is a tendency for such material to "float." The 10 per cent of patent red lining will be a factor in causing the finish, resulting from this powder, to be coarse and rough. Moreover, the patent color will fade upon exposure to strong light for any length of time. Since the dye used in coloring the patent color is soluble in many of the solvents used in clear gloss lacquers, it will bleed into the top coat which is applied over the coat of bronzing lacquer. This is a desirable feature, but it is difficult to control since different spray operators apply the material differently. This tends toward a lack of color uniformity in production.

Oxidized pale gold powders, which have the disadvantages previously mentioned, constitute 50 per cent of the powder and will cause the finish to be coarse and porous. The 20 percent of oxidized rich gold powder has the same qualities. The remaining 15 per cent of the powder consists of a straight-run copper powder. Since this powder is of a fine texture it will tend to make the finish smooth and dense, but since it is in less proportion than the other powders, its advantages are nullified.

35 A bronze powder paste embodying the present invention and which duplicates the above mentioned powder in shade consists of:

|                                  | Per cent |
|----------------------------------|----------|
| Straight-run copper fine         | 31.77    |
| Straight-run green gold          | 23.56    |
| Carbon black                     | 5.09     |
| Lithol red                       | 1.14     |
| Coumarone-indene resin           | 21.86    |
| Hi-flash naphtha                 | 15.79    |
| Rezyl 869 (long oil alkyd resin) | .79      |

This paste will have a greater coverage than a powder of corresponding color. This paste will cover 400 square feet per gallon when mixed with 50 a bronzing lacquer, for example, a lacquer comprising 12½ per cent 6 sec. bronzing nitro-cellulose in lacquer thinner, with 4½ fluid ounces of plasticizer and 8 fluid ounces of a medium long drying type alkyd resin to a gallon. The corresponding powder when mixed with the same ve-

hicle at the same ratio, i. e., one pound of powder per gallon will cover 225 square feet per gallon. The film resulting from the paste is much smoother than that from the powder. The gloss lacquer top coat does not need to be applied nearly as heavily on the paste film as on the powder in order to get a gloss.

The invention consists principally in a paste wherein the unoxidized bronze powder is mixed with alkyd resin of low acid number and a non-acid volatile thinner that is free from sulphur, with or without pigment. It also consists in the compositions and process of making same herein-after described and claimed.

According to the present invention, I use straight run bronze powder made as heretofore by grinding and polishing the metal aluminum, copper or zinc or alloys thereof into small particles, such say, as will pass a No. 100 or finer mesh screen. This straight run powder carries a small quantity of non-acid grease, preferably stearic acid that was mixed with the metal particles at the rate of from four to eight ounces per hundred pounds of metallic powder in the process of grinding for the purpose of polishing the same.

This polished metal powder is used without any treatment by heat or otherwise that would cause any oxidation or change of color or that would affect the thin, flat shape of the particles. This metal powder is mixed with alkyd resin and low boiling point naphtha, together with a suitable pigment. The following is a typical example, namely, unoxidized copper metal powder about 55 per cent, alkyd resin of low acid number, say lower than 8, about 17 per cent Hi-flash naphtha free from sulphur and acidity about 18 per cent, lamp black 9.75 per cent and organic lithol-red .32 per cent. This composition is in the form of a soft paste suitable for packaging and easy to dispense in desired quantities. The naphtha is used as a volatile thinner and its quantity is subject to considerable variation. The alkyd resin is the vehicle or carrier for the metallic particles and other pigment, with which it is quite compatible and which it preserves against oxidation and sulphidizing. A special advantage of alkyd resin is that it is exceptionally well adapted for grinding and for mixing with the other ingredients of my composition and preserves the color and luster of the metal particles unimpaired. The term "acid number" as applied to resin is the number of milligrams of potassium hydroxide that are required to neutralize one gram of the particular oil or resin under question; for example, if one gram of a resin requires 3 milligrams of potassium hydroxide to neutralize it, then the resin is said to have an acid number of 3.

The quantities of metallic particles, lamp black and other pigments are subject to considerable variations, as the color effects vary with the selection of pigments and the proportions in which they are mixed. It is a great advantage of the present invention that such selections and mixtures can be made by skilled artisans at the factory and with the assurance that all lots made in accordance with a given formula will match even though they may not be used for considerable periods of time.

In the example specified, about ten per cent of the composition consists of lamp black which is used as a pigment and which might have been omitted entirely if it has been desired to bring out the light tones of the metal.

The following resins are all adapted for the

practice of my invention: pure alkyd resins, as Beckosol No. 1323 and Beckosol No. 1307, phenol modified alkyd resins, as Beckosol No. 1320, oil and phenol modified resins, as Beckosol No. 1, coumarone-indene resins, as cumar, phenol modified coumarone-indene resins, as Nevillac and pure phenolic resins, as Beckacite No. 2000.

The paste hereinbefore described is a rather concentrated preparation and preferably contains all desired pigment so as to be ready for addition to any of the usual varnishes or lacquers. I have found that varnish and lacquer embodying my composition produces a smoother coat and has greater covering capacity than varnish or lacquer that embodies bronze powders heat treated to produce substantially the same color effect. I have found also that varnishes and lacquer embodying my composition require a thinner surface or finish coat of clear lacquer or varnish than is required for other varnishes.

What I claim is:

1. A bronze paste consisting of straight run bronze powder, resin of acid number lower than 8 and a volatile thinner free of sulphur and acidity.
2. A bronze paste consisting of straight run bronze powder, resin of acid number lower than 8 and a volatile thinner free of sulphur and acidity.
3. A bronze paste consisting of straight run bronze powder, at least two resins of acid number lower than 8 and volatile thinner free of sulphur and acidity.
4. A bronze paste consisting of polished bronze powder in the form of thin flat particles, resin of acid number lower than 8, a volatile thinner free of sulphur and acidity, and pigment.
5. A bronze paste consisting of straight run bronze powder, resin of acid number lower than 8 and a volatile thinner free of sulphur and acidity, together with pigment.
6. A bronze paste comprising unoxidized bronze powder in the form of thin flat particles, resin of acid number lower than 8, a volatile thinner free of sulphur and acidity, lamp black and other pigment.
7. A bronze paste consisting mainly of polished metallic copper powder in the form of thin flat particles free from oxide and sulphide discoloration, resin of acid number lower than 8, and naphtha free of sulphur and acidity.
8. A bronze paste consisting mainly of polished metallic copper powder in the form of thin flat particles free from oxide and sulphide discoloration, coumarone-indene resin and an alkyd resin of acid number lower than 8, and naphtha free of sulphur and acidity.
9. A bronze paste consisting mainly of straight run metallic copper powder in the form of thin flat particles free from oxide and sulphide discoloration, alkyd resin of acid number lower than 8 and naphtha free of sulphur and acidity, in substantially the proportions of three parts of straight run powder to one part of alkyd resin and one part of naphtha.
10. A bronze paste consisting mainly of polished metallic copper powder in the form of thin flat particles free from oxide and sulphide discoloration, alkyd resin of acid number lower than 8 and naphtha free of sulphur and acidity, in substantially the proportions of three parts of powder to one part of alkyd resin and one part of naphtha.
11. A bronze paste comprising unoxidized bronze powder in the form of thin flat particles,

alkyd resin of acid number lower than 8, and naphtha free of sulphur and acidity, in substantially the proportion of 55 parts of bronze powder to 17 parts of alkyd resin and 18 parts of naphtha together with pigment.

12. A bronze paste comprising unoxidized bronze powder in the form of thin flat particles,

alkyd resin of acid number lower than 8, and naphtha free of sulphur and acidity, and lamp black, in substantially the proportion of 55 parts of bronze powder to 17 parts of alkyd resin, 18 parts of naphtha and 10 parts of lamp black.

LEO J. MITCHELL.